# EUROPEAN PATENT SPECIFICATION

(11) **EP 0 144 793 B1**
(45) Date of publication and mention of the grant of the patent: **12.10.1988**
(21) Application number: 84113512.2
(22) Date of filing: 09.11.1984
(51) Int. Cl.: D01F 6/18, D01D 5/00

(54) **High tenacity and modulus polyacrylonitrile fiber and method**
Polyacrylnitrilfaser mit hoher Festigkeit und hohem Modul und Verfahren zur Herstellung derselben
Fibre en polyacrylonitrile à haute ténacité et haut module, et procédé de fabrication

(30) Priority: 05.12.1983 US 557984
(43) Date of publication of application: 19.06.1985
(73) Proprietor: AlliedSignal Inc., Morristown, New Jersey 07962-2245 (US)
(72) Inventor: Kwon, Young D., Morristown, NJ 07960 (US); Kavesh, Sheldon, Morristown, NJ 07960 (US); Prevorsek, Dusan C., Morristown, NJ 07960 (US)
(74) Representative: Brock, Peter William

(56) References cited:
- EP-A- 0 044 534
- FR-A- 2 405 275
- GB-A- 1 100 497
- US-A- 4 344 908

## Description

The present invention relates to a process for preparing polyacrylonitrile (PAN) fibers and fibers as produced, and especially to such a process and fiber product employing PAN of ultrahigh moelcular weight.

PAN has been spun conventionally using either wet spinning (e.g., 9.5% PAN in sodium thiocyanate- water (50:50) spun into 10% sodium thiocyanate in water at -2°C for coagulation) or dry spinning (e.g., 30% PAN in diethylformamide spun at 130°C). Typical properties of the resultant fibers are 2.4-3.7 g/denier (21.168 to 32.634 cN/tex) tenacity and 42-53 g/denier (370.44 to 467.46 cN/tex) tensile modulus. See Table 1 on page 155 of S.S. Chari et al., Fibre Science and Technology, Vol. 15, pp. 153-60 (1981). Mention is also made of PAN fibers in U.S. patent 4,344,908 to Smith et. al. (1982) concerned primarily with polyethylene fibers. Also concerned primarily with polyethylene fibers is U.S. Patent 4,413,110 of Kavesh and Prevorsek (November 1, 1983).

EP 0,044,534A discloses both wet spinning and dry spinning processes for producing polyacrylonitrile filaments and fibers having an initial modulus based on 100% elongation of greater than 1,300 cN/tex. The polymers used may have relative solution viscosities (0.5% concentration in dimethyl formamide) in the range 1.7 to 6.0.

### Brief description of the invention

The present invention relates to a gel-spinning process employing a polyacrylonitrile of very high molecular weight. Unlike wet-spinning (coagulation) processes, in gel spinning, the spun solution is cooled to below the gelling temperature before extraction of the spinning solvent.

Thus, the present invention provides a gel-spinning process comprising the steps:
(a) forming a solution of a substantially linear polyacrylonitrile having a weight average molecular weight of least 500,000 in a first solvent at a first concentration of 2 to 15 weight percent polyacrylonitrile, and at a first temperature above the gelation temperature said solvent having a vapor pressure of no more than 80 kPa at said first temperature,
(b) extruding said solution through an aperture into a gaseous atmosphere, the extruded solution being at a temperature above the gelation temperature and the concentration of polyacrylonitrile being substantially at the first concentration both upstream and downstream of said aperture,
(c) cooling the solution in a cooling zone adjacent to and downstream of the gaseous atmosphere to a second temperature below the gelation temperature to form a rubbery gel containing first solvent of substantially indefinite length,
(d) extracting the gel containing first solvent with a second solvent which is more volatile than said first solvent for a sufficient contact time to form a fibrous structure containing second solvent, which fibrous structure is substantially free of first solvent and is of substantially indefinite length,
(e) drying the fibrous structure containing second solvent to form a xerogel of substantially indefinite length free of first and second solvent, and
(f) stretching at least one of:
   (i) the gel containing the first solvent,
   (ii) the fibrous structure containing the second solvent, and
   (iii) the xerogel, at a total stretch ratio sufficient to achieve a tenacity of at least 5 g/denier (44.1 cN/tex) and a secant modulus of at least 100 g/denier (882 cN/tex).

The present invention also includes a polyacrylonitrile fiber of weight average molecular weight at least 500,000 and having a tenacity of at least 5 g/denier (44.1 cN/tex) and a secant modulus of at least 100 g/denier (882 cN/tex). Such fibers are useful in tire cord and in the preparation of carbon fibers, especially for composites.

### Detailed description of the invention

The process and fibers of the present invention employ a linear ultrahigh molecular weight polyacrylonitrile (PAN) described more fully below that enables the preparation of PAN fibers of heretofore unobtained properties by extrusion of dilute solutions of concentration lower than used in Wet Spinning or Dry Spinning. Furthermore, the preferred solvents of the present invention do not phase-separate from PAN on cooling to form a non-PAN coating or occluded phase, but rather form a dispersed fairly homogeneous gel.

The PAN polymer used is substantially linear and of weight average molecular weight at least 500,000, preferably at least 750,000, more preferably between 1,000,000 and 4,000,000 and most preferably between 1,500,000 and 2,500,000.

Such substantially linear ultrahigh molecular weight PAN can be prepared by the procedures illustrated in Preparations A and B immediately proceeding Example 1, below. While ultrahigh molecular weight PAN is known (see U.S. patent 4,254,250 Col. 5, Table I), its prior use was in preparing water treatment polymers.

The first solvent should have a vapour pressure of no more than 80 kPa at said first temperature. This is necessary in order to maintain essentially constant the concentration of solvent upstream and through the aperture (die) and to prevent non-uniformity in liquid content of the gel fiber or film containing first solvent. Preferably, the vapor pressure of the first solvent should be no more than 80 kPa (four-fifths of an atmosphere) at 130°C. Suitable first solvents for PAN include dimethylsulfoxide (DMSO), dimethylformamide (DMF), dimethylacetamide (DMAc), gamma-butyrolactone and ethylene carbonate. Other homologs and analogs of these solvents (e.g., propylene carbonate) may also be used. Less preferred are aqueous solutions of salts such as concentrated aqueous sodium thiocyanate. DMSO is most preferred.

The polymer is present in the first solvent at a first concentration of 2 to 15 weight percent, preferably 4 to 10 weight percent more preferably 5 to about 8 weight percent; however, once chosen, the concentration should not vary significantly adjacent the die or otherwise prior to cooling to the second temperature. The concentration at any one point should not vary adjacent the die or otherwise prior to cooling to the second temperature. The concentration should also remain reasonably constant over time (i.e. length of the fiber or film).

The first temperature is chosen to achieve complete dissolution of the polymer in the first solvent. The first temperature is the minimum temperature at any point between where the solution is formed and the die face, and must be greater than the gelation temperature for the polymer in the solvent at the first concentration. For PAN in DMSO at 5-8% concentration, the gelation temperature is approximately 25-100°C; therefore, a preferred first temperature can be about 130°C to about 200°C, more preferably about 140-180°C. While temperatures may vary above the first temperature at various points upstream of the die face, excessive temperatures causative of polymer degradation should be avoided. To assure complete solubility, a first temperature is chosen whereat the solubility of the polymer exceeds the first concentration and is typically at least 20% greater. The second temperature is chosen whereat the first solvent-polymer system behaves as a gel, i.e., has a yield point and reasonable dimensional stability for subsequent handling. Cooling of the extruded polymer solution from the first temperature to the second temperature should be accomplished at a rate sufficiently rapid to form a gel fiber which is of substantially the same polymer concentration as existed in the polymer solution. Preferably the rate at which the extruded polymer solution is cooled from the first temperature to the second temperature should be at least 50°C per minute.

A preferred means of cooling to the second temperature involves the use of a quench bath. The quench bath will preferably comprise a mixture of the first solvent with water. The water concentration of the quench bath may range from about 0 to about 95%. The quench bath may also comprise a liquid which is relatively immiscible with the first solvent. Suitable liquids include soybean oil, silicon oil, etc. Quenching temperatures that may be employed range from about 0°C to about 50°C with a temperature near room temperature being preferred.

Some stretching during cooling to the second temperature is not excluded from the present invention, but the total stretching during this stage should not normally exceed 10:1. As a result of those factors the gel fiber formed upon cooling to the second temperature consists of a continuous polymeric network highly swollen with solvent.

If an aperture of circular cross section (or other cross section without a major axis in the plane perpendicular to the flow direction more than 8 times the smallest axis in the same plane, such as oval, Y-or X- shaped aperture) is used, then both gels will be gel fibers, the xerogel will be a xerogel fiber. The diameter of the aperture is not critical, with representative apertures being between 0.25 mm and 5 mm in diameter (or other major axis). The length of the aperture in the flow direction should normally be at least 10 times the diameter of the aperture (or other similar major axis), preferably at least 15 times and more preferably at least 20 times the diameter (or other similar major axis).

If an aperture of rectangular cross section is used, then both gels will be gel films, the xerogel will be a xerogel film and the thermoplastic article will be a film. The width and height of the aperture are not critical, with representative apertures being between 2.5 mm and 2 m in width (corresponding to film width), between 0.25 mm and 5 mm in height (corresponding to film thickness). The depth of the aperture (in the flow direction) should normally be at least 15 times the height and more preferably at least 20 times the height.

The extraction with second solvent is conducted in a manner that replaces the first solvent in the gel with a second more volatile solvent. When the first solvent is DMSO or DMF, a suitable second solvent is water. Preferred second solvents are the volatile solvents having an atmospheric boiling point of 100°C or lower. Conditions of extraction should remove the first solvent to less than 1 % solvent by weight of polymer in the gel after extraction.

With some first solvents such as DMSO or DMF, it is contemplated (but not preferred) to evaporate the solvent from the gel fiber near the boiling point of the first solvent and/or at subatmospheric pressure instead of or prior to extraction.

A preferred combination of conditions is a first temperature between 130°C and 250°C, a second temperature between 0°C and 50°C and a cooling rate of at least 50°C/minute. The first solvent should have a vapor pressure at the first temperature of less than four-fifths atmosphere (80 kPa). In choosing the first and second solvents, the primary desired difference relates to volatility as discussed above.

Once the fibrous structure containing second solvent is formed, it is then dried under conditions where the second solvent is removed leaving the solid network of polymer substantially intact. By analogy to silica gels, the resultant material is called herein a "xero-gel" meaning a solid matrix corresponding to the solid matrix of a wet gel, with the liquid replaced by gas (e.g. by an inert gas such as nitrogen or by air). The term "xerogel" is not intended to delineate any particular type of surface area, porosity or pore size.

Stretching may be performed upon the gel fiber after cooling to a second temperature or during or after extraction. Alternatively, stretching of the xerogel fiber may be conducted, or a combination of gel stage stretching may be conducted in a single stage or it may be conducted in two or more stages. The first stage stretching may be conducted at room temperature or at an elevated temperature. Preferably the stretching is conducted in two or more stages with the last of the stages performed at a temperature between 100°C and 250°C. Most preferably the stretching is conducted in at least two stages with the last of the stages performed at a temperature between 130°C and 230°C.

Such temperatures may be achieved with heated tubes as in the Figures, or with other heating means such as heating blocks or steam jets.

The product PAN fibers produced by the present process represent novel articles in that they include fibers with a unique combination of properties: a molecular weight of at least 500,000, a (secant) modulus at least 100 g/denier (882 cN/tex) and a tenacity at least 5 g/denier (44.1 cN/tex). For this fiber, the molecular weight is preferably at least 750,000, more preferably between 1,000,000 and 4,000,000 and most preferably between 1,500,000 and 2,500,000. The tenacity is preferably at least 7 g/denier (61.74 cN/tex). The secant modulus is preferably at least 100 g/denier (882 cN/tex), more preferably at least 125 g/denier (1102.5 cN/tex). Preferably the fiber has an elongation to break at most 7%.

### Description of the preferred embodiments

Figure 1 illustrates in schematic form a first embodiment of the present invention, wherein the stretching step F is conducted in two stages on the xerogel fiber subsequent to drying step E. In Figure 1, a first mixing vessel 10 is shown, which is fed with an ultra high molecular weight polymer 11 such as PAN of weight average molecular weight at least 500,000 and frequently at least 750,000, and to which is also fed a first, relatively non-volatile solvent 12 such as DMSO. First mixing vessel 10 is equipped with an agitator 13. The residence time of polymer and first solvent in first mixing vessel 10 is sufficient to form a slurry containing some dissolved polymer and some relatively finely divided polymer particles, which slurry is removed in line 14 to an intensive mixing vessel 15. Intensive mixing vessel 15 is equipped with helical agitator blades 16. The residence time and agitator speed in intensive mixing vessel 15 is sufficient to convert the slurry into a solution. It will be appreciated that the temperature in intensive mixing vessel 15, either because of external heating, heating of the slurry 14, heat generated by the intensive mixing, or a combination of the above is sufficiently high (e.g. 150°C) to permit the polymer to be completely dissolved in the solvent at the desired concentration (generally between 5 and 10 percent polymer by weight of solution). From the intensive mixing vessel 15, the solution is fed to an extrusion device 18, containing a barrel 19 within which is a screw 20 operated by motor 22 to deliver polymer solution at reasonably high pressure to a gear pump and housing 23 at a controlled flow rate. A motor 24 is provided to drive gear pump 23 and extrude the polymer solution, still hot, through a spinnerette 25 comprising a plurality of aperatures, which may be circular, X-shaped, or, oval-shaped, or in any of a variety of shapes having a relatively small major axis in the plane of the spinnerette when it is desired to form fibers, and having a rectangular or other shape with an extended major axis in the plane of the spinnerette when it is desired to form films. The temperature of the solution in the mixing vessel 15, in the extrusion device 18 and at the spinnerette 25 should all equal or exceed a first temperature (e.g. 150°C) chosen to exceed the gellation temperature (approximately 0-100⁰C for PAN in DMSO). The temperature may vary (e.g. 140°C, 160°C) or may be constant (e.g. 150°C) from the mixing vessel 15 to extrusion device 18 to the spinnerette 25. At all points, however, the concentration of polymer in the solution should be substantially the same. The number of apertures, and thus the number of fibers formed, is not critical, with convenient numbers of apertures being 16, 120, or 240.

From the spinnerette 25, the polymer solution passes through an air gap 27, optionally enclosed and filled with an inert gas such as nitrogen, and optionally provided with a flow of gas to facilitate cooling. A plurality of gel fibers 28 containing first solvent pass through the air gap 27 and into a quench bath 30 containing any of a variety of liquids, so as to cool the fibers, both in the air gap 27 and in the quench bath 30, to a second temperature such that the polymer-solvent system forms a gel. It is preferred that the quench liquid in quench batch 30 be a mixture of first solvent (DMSO) and water. While some stretching in the air gap 27 and in the quench medium is permissible, it is preferably less than about 10:1. Rollers 31 and 32 in the quench bath 30 operate to feed the fiber through the quench bath, and preferably operate with little or no stretch.

From the quench bath 30, the cool first gel fibers 33 pass (preferably with some room temperature stretching) to a solvent extraction device 37 where a second solvent, being of relatively low boiling temperature such as water, is fed through line 38. The solvent outflow in line 40 contains second solvent and essentially all of the first solvent brought in with the cool gel fibers 33, either dissolved or dispersed in the second solvent. Thus the fibrous structure 41 conducted out of the solvent extraction device 37 contains substantially only second solvent, and relatively little first solvent. The fibrous structure 41 may have shrunken somewhat compared to the first gel fibers 33.

In a drying device 45, the second solvent is evaporated from the fibrous structure 41, forming essentially unstretched xerogel fibers 47 which are taken up on spool 52.

From spool 52, or from a plurality of such spools if it is desired to operate the stretching line at a slower feed rate than the take up of spool 52 permits, the fibers are fed over driven feed roll 54 and idler roll 55 into a first heated tube 56, which may be rectangular, cylindrical or other convenient shape. Sufficient heat is applied to the tube 56 to cause the fiber temperature to be between 100-200°C. The fibers are stretched at a relatively high draw ratio (e.g. 4: 1) so as to form partially stretched fibers 58 taken up by driven roll 61 and idler roll 62. From rolls 61 and 62, the fibers are taken through a second heated tube 63, heated so as to be at somewhat higher temperature, e.g. 130-230°C and are then taken up by driven take-up roll 65 and idler roll 66, operating at a speed sufficient to impart a stretch ratio in heated tube 63 as desired, e.g. 1.8: 1. The twice stretched fibers 68 produced in this first embodiment are taken up on take-up spool 72. It is anticipated that some or all of the stretch ratios may be decreased as the line speeds are increased.

With reference to the six process steps of the present invention, it can be seen that the solution forming step A is conducted in mixers 13 and 15. The extruding step B is conducted with device 18 and 23, and especially through spinnerette 25. The cooling step C is conducted in airgap 27 and quench bath 30. Extraction step D is conducted in solvent extraction device 37. The drying step E is conducted in drying device 45. The stretching step F is conducted in elements 52-72, and especially in heated tubes 56 and 63. It will be appreciated, however, that various other parts of the system may also perform some stretching, even at temperatures substantially below those of heated tubes 56 and 63. Thus, for example, some stretching (e.g. 1.5:1 to 5:1) may occur within quench bath 30, between the quench bath 30 and the solvent extraction device 37, within solvent extraction device 37, within drying device 45 or between solvent extraction device 37 and drying device 45.

A second embodiment of the present invention is illustrated in schematic form by Figure 2. The solution forming and extruding steps A and B of the second embodiment are substantially the same as those in the first embodiment illustrated in Figure 1. Thus, polymer and first solvent are mixed in first mixing vessel 10 and conducted as a slurry in line 14 to intensive mixing device 15 operative to form a hot solution of polymer in first solvent. Extrusion device 18 impells the solution under pressure through the gear pump and housing 23 and then through a plurality of apertures in spinnerette 27. The hot first gel fibers 28 pass through air gap 27 and quench bath 30 so as to form cool first gel fibers 33.

The cool first gel fibers 33 are conducted over driven roll 54 and idler roll 55 through heated tube 57 which, in general, is longer than the first heated tube 56 illustrated in Figure 5. The fibers 33 are drawn through heated tube 57 by driven take-up roll 59 and idler roll 60, so as to cause a relatively high stretch ratio (e.g. 10:1). The once-stretched first gel fibers 35 are conducted into extraction device 37.

In the extraction device 37, the first solvent is extracted out of the gel fibers by second solvent and the fibrous structures 42 containing second solvent are conducted to a drying device 45. There the second solvent is evaporated from the fibrous structures; and xerogel fibers 48, being once-stretched, are taken up on spool 52.

Fibers on spool 52 are then taken up by driven feed roll 61 and idler 62 and passed through a heated tube 63, operating at the relatively high temperature of between 150 and 270°C. The fibers are taken up by driven take up roll 65 and idler roll 66 operating at a speed sufficient to impart a stretch in heated tube 63 as desired, e.g. 1.8:1. The twice-stretched fibers 69 produced in the second embodiment are then taken up on spool 72.

It will be appreciated that, by comparing the.embodiment of Figure 2 with the embodiment of Figure 1, the stretching step F has been divided into two parts, with the first part conducted in heated tube 57 performed on the first gel fibers 33 prior to extraction (D) and drying (E), and the second part conducted in heated tube 63, being conducted on xerogel fibers 48 subsequent to drying (E).

The third embodiment of the present invention is illustrated in Figure 3, with the solution forming step A, extrusion step B, and cooling step C being substantially identical to the first embodiment of Figure 1 and the second embodiment of Figure 2. Thus, polymer and first solvent are mixed in first mixing vessel 10 and conducted as a slurry in line 14 to intensive mixing device 15 operative to form a hot solution of polymer in first solvent. Extrusion device 18 impells the solution under pressure through the gear pump and housing 23 and then through a plurality of apertures in spinnerette 27. The hot first gel fibers 28 pass through air gap 27 and quench bath 30 so as to form cool first gel fibers 33.

The cool first gel fibers 33 are conducted over driven roll 54 and idler roll 55 through a heated tube 57 which, in general, is longer than the first heated tube 56 illustrated in Figure 5. The length of heated tube 57 compensates, in general, for the higher velocity of fibers 33 in the third embodiment of Figure 7 compared to the velocity of xerogel fibers (47) between take-up spool 52 and heated tube 56 in the first embodiment of Figure 1. The first gel fibers 33 are now taken up by driven roll 61 and idler roll 62, operative to cause the stretch ratio in heated tube 57 to be as desired, e.g. 5:1.

From rolls 61 and 62, the once-drawn first gel fibers 35 are conducted into modified heated tube 64 and drawn by driven take up roll 65 and idler roll 66. Driven roll 65 is operated sufficiently fast to draw the fibers in heated tube 64 at the desired stretch ratio, e.g. 1.8:1. Because of the relatively high line speed in heated tube 64, required generally to match the speed of once-drawn gel fibers 35 coming off of rolls 61 and 62, heated tube 64 in the third embodiment of Figure 3 will, in general, be longer than heated tube 63 in either the second embodiment of Figure 2 or the first embodiment of Figure 1. While first solvent may exude from the fiber during stretching in heated tubes 57 and 64 (and be collected at the exit of each tube), the first solvent is sufficiently non-volatile so as not to evaporate to an appreciable extent in either of these heated tubes.

The twice-stretched first gel fiber 36 is then conducted through solvent extraction device 37, where the second, volatile solvent extracts the first solvent out of the fibers. The fibrous structures 43, containing substantially only second solvent, are then dried in drying device 45, and the twice-stretched fibers 70 are then taken up on spool 72.

It will be appreciated that, by comparing the third embodiment of Figure 3 to the first two embodiments of Figures 1 and 2, the stretching step (F) is performed in the third embodiment in two stages, both subsequent to cooling step C and prior to solvent extracting step D.

The present polyacrylonitrile fibers may be used as such in tire cord and other applications. In addition, they may be carbonized or graphitized, in the manner conventionally employed for polyacrylonitrile fibers (see Kirk-Othmer, Encyclopedia of Chemical Technology, vol. 4, pp. 625-26 (1978); British Patent 1,110,791 (April 24, 1968)) and the above-cited Chari et al article) to produce carbon fibers of superior properties.

The polyacrylonitrile used in the following Examples was prepared by the procedure illustrated below in Preparation C.

### Preparation A

The reactor consisted of a 1-liter, 3-neck, round-bottom flask with indented wall. It was fitted with a stirrer, a condenser, and a stopper. The flask is placed in a constant temperature bath at 35°C. It was evacuated and filled with oxygen-free nitrogen four times using a Firestone valve. The system was blanketed with nitrogen throughout the polymerization period.

A mixture of 300 mL freshly boiled, deionized, and distilled water, 3 g of sodium lauryl sulfate, and 2 mL of 0.1N H_{Z}S0₄ solution was added and stirred. To this was added 100 mL (80 g) of redistilled acrylonitrile and stirred vigorously to form an emulsion. After 5 minutes, 0.2 g of potassium persulfate and 0.08 g of sodium metabisulfite were added. The mixture was stirred for 22 hours under nitrogen. The emulsion formed was mixed with 600 mL of methanol with stirring. The polymer precipitated was isolated by filtration. It was purified by washing twice using hot water (50-60°C) with vacuum filtration, followed by drying to a constant weight. There was obtained 78 g (98% yield) of polyacrylonitrile having an intrinsic viscosity of 9.92 dUg when determined in N,N-dimethylformamide at 35°C. This was calculated to have an estimate molecular weight of 1.06x10⁶ using the following equation:

### Preparation B

A similar procedure was used in this experiment. A 500-ml flask was charged with a mixture of 150 mL of deaerated, deionized, and distilled water, 1.5 g sodium lauryl sulfate, 1 mL of 0.1 N H_{z}S0₄, 50 mL of redistilled acrylonitrile, 0.1 g of K₂S₂0, and 0.04 g of Na₂S₂₀ₛ, in that order.

After stirring for 1 hour at 35°C, another batch of 0.1 g K₂S₂0₈ and 0.04 g of Na₂S20₅ was added. The mixture was stirred vigorously under nitrogen for four more hours and then treated with methanol. The precipitated polymer was filtered, washed twice with hot water, and dried. There was obtained 37.1 g (93% yield) of polyacrylonitrile.

The intrinsic viscosity was found to be 5.67 dUg when measured in N,N - dimethylformamide at 35°C. On the basis described in Preparation A, this corresponds to an estimated molecular weight of 5.5x10^{s}.

### Preparation C

A 500 ml 3-neck flask equipped with a stirrer, a condenser and a stopper was flushed well and blanketed with nitrogen. A mixture containing 120 ml of deaerated, deionized water, 2 g of sodium lauryl sulfate, 80 g of purified acrylonitrile, 0.1 g of potassium persulfate, and 0.03 g of sodium metabisulfite, was added. The mixture was stirred vigorously at 35°C for 1 hour. Another batch of 0.1 g of potassium persulfate and 0.03 g of sodium metabisulfate was added. After stirring for 24 hours under an atmosphere of nitrogen, the mixture was mixed with 1.5 L of water and 150 g of sodium chloride. The polymer formed was obtained by filtration and then washed four times with water until the filtrate was free of chloride. The polyacrylonitrile was collected by filtration and dried in air at room temperature. Its intrinsic viscosity was found to be 13.65 dUg when measured in N,N - dimethylformamide at 35°C. This was calculated to have an estimated molecular weight of 1.63x10⁶ using the equation given in Preparation A.

The process of the invention will be illustrated by the examples below.

### Examples

The modulus values reported in Example 1-4 represent secant modulus (the slope of a chord on the stress-strain curve drawn between the origin and the breaking point). Such secant modulus values are normally lower than the initial modulus, in some cases by a factor of 2. Selected fibers were also evaluate for initial modulus, and both values are given in Table 1 at the end of the Examples.

### Example 1

An Atlantic Research Corporation Model 2CV Helicone@ mixer charged with a 6.0 weight percent solution of the PAN prepared in Preparation C, having a molecular weight of approximately 1.63x 10", and 94 weight percent dimethyl sulfoxide. The charge was heated with agitation at 12 rev/min at 25°C under nitrogen pressure for two hours and then for two hours at 145°C.

The solution was extruded at the final mixing temperature (i.e. 145°) through a 0.030 inch (0.762 mm) diameter aperture (UD=25) at a reasonably constant rate of 2.03 cm³/min.

The extruded uniform solution filament was quenched to a gel state by passage through a bath comprising 50 weight percent water and 50 weight percent dimethyl sulfoxide, said bath being located 1 cm below the spinning die. The gel filament was wound up continuously on a 6.5 cm diameter, 20.4 cm long bobbin at the rate of 599 cm/min.

The gel fiber was then kept in a stirred water bath having a temperature of 22°C for 18 hours in order to extract the dimethyl sulfoxide from the fiber. Thereafter, the fiber was dried at a temperature of 25°C. Drying of the fiber was accomplished by leaving in air at room temperature.

The dried fiber was then drawn via a two stage drawing process. First stage drawing was accomplished by feeding the fiber at a speed of 118 cm/min into a hot tube, five-eighths inch (14 mm) inside diameter, and 6 feet (180 cm) in length, blanketed with nitrogen. The temperature at the entrance of the hot tube being 135°C with the exit temperature of the hot tube being 150°C. The fiber was drawn at a ratio of 4.07/1 within the tube. Second stage drawing of the once stretched fiber was accomplished by drawing the fiber in the same tube wherein the fiber was fed into the tube at a speed of 215 cm/min, with the tube entrance temperature being 146°C, the tube exit temperature being 160°C, and the drawing ratio being 2.11/1. The properties of the twice stretched fibers was as follows:
denier: 10.5
tenacity: 7.8 g/denier (68.8 cN/tex)
secant modulus: 138 g/denier (1217.16 cN/tex)
ultimate elongation: 5.8

### Example 2

Example 1 was repeated with 6% PAN in DMSO and the extrusion rate lowered from 2.03 to 1.97 cm³/min and the take-up speed raised from 599 cm/min to 605 cm/min (so as to produce a die-draw of 1.4:1 instead of 1.35:1). Six sets of fibers were prepared using various first stretch conditions (tube temperature, draw ratio, draw duration) as follows:

Fiber properties were measured (4 replications) on such once-drawn fibers, and are indicated below, with average values indicated, followed by maximum values in parentheses:

The once-drawn fibers were then drawn again under conditions indicated below:

The properties of the twice-stretched fibers were then measured (at least three replications), with the results indicated below:

### Example 3

Example 1 was repeated, now mixing the PAN to 6.0% concentration in gamma-butyrolactone for four hours at 145°C. Spinning was at 145°C, at 2.17 mUmin into water-methanol (50:50). Take-up speed was 617 cm/min (1.3:1 die-draw). The fibers were extracted at 22°C for 18 hours in stirred methanol. The fibers were twice drawn as follows:

Properties of selected fibers were measured on an Instron@ tensile testing machine as follows:

### Example 4

Example 1 was repeated using 6.0% PAN in dimethyl formamide, mixed at 145°C for four hours. Spinning through the 0.030 inch (0.78 mm) diameter die was at 133°C at 1.96 mL min with take-up at 519 cm/min (1.20:1 die-draw). Extraction was in water for 17 hours with stirring and then 4 hours without stirring. Two stage drawing was as follows:

Fiber properties were determined (one replication for the three once-drawn fibers, four replications for the six twice-drawn fibers) as follows:

The following table illustrates the relation between initial modulus and secant modulus for selected fibers (six individual fibers indicated above as 2B2):

Testing was conducted on an Instron machine with 5 inch (12.7 cm) sample lengths and a 5 inch/min (12.7 cm/min) head speed. Elongations were on the order of 0.3 inch (0.8 cm) or approximately 6%.

## Claims

1. A gel-spinning process for preparing a polyacrylonitrile fiber comprising the steps:
(a) forming a solution of a substantially linear polyacrylonitrile having a weight average molecular weight of at least 500,000 in a first solvent at a first concentration of 2 to 15 weight percent polyacrylonitrile, and at a first temperature above the gelation temperature said solvent having a vapor pressure of no more than 80 kPa at said first temperature,
(b) extruding said solution through an aperture into a gaseous atmosphere, the extruded solution being at a temperature above the gelation temperature and the concentration of polyacrylonitrile being substantially at the first concentration both upstream and downstream of said aperture,
(c) cooling the solution in a cooling zone adjacent to and downstream of the gaseous atmosphere to a second temperature below the gelation temperature to form a rubbery gel containing first solvent of substantially indefinite length,
(d) extracting the gel containing first solvent with a second solvent which is more volatile than said first solvent for a sufficient contact time to form a fibrous structure containing second solvent, which fibrous structure is substantially free of first solvent and is of substantially indefinite length,
(e) drying the fibrous structure containing second solvent to form a xerogel of substantially indefinite length free of first and second solvent, and
(f) stretching at least one of:
(i) the gel containing the first solvent,
(ii) the fibrous structure containing the second solvent, and
(iii) the xerogel, at a total stretch ratio sufficient to achieve a tenacity of at least 5 g/denier (44.1 cN/tex) and a secant modulus of at least 100 g/denier (882 cN/tex).

2. The process of claim 1 wherein said aperture has an essentially circular cross-section; said gel containing first solvent is a gel fiber; said xerogel is a xerogel fiber.

3. The process of claim 1 or 2 wherein said first temperature is between 130°C and 250°C; said second temperature is between 0°C and 50°C; and the cooling rate between said first temperature and said second temperature is at least 50°C/min.

4. The process of any previous claim wherein said second solvent has an atmospheric boiling point of 100°C or lower.

5. The process of any previous claim wherein said first solvent is selected from the group consisting of dimethylsulfoxide, dimethylformamide, dimethylacetamide, gamma butyrolactone and ethylene carbonate.

6. The process of any of claims 1-3 wherein said first solvent is dimethylsulfoxide, said first temperature is 130°C to 200°C and said first concentration is 5 to 8 weight percent.

7. The process of any previous claim wherein said stretching step (f) is conducted in at least two stages.

8. The process of claim 7 wherein a first stretching stage is of the gel containing the first solvent.

9. The process of claim 8 wherein a second stretching stage is of the xerogel.

10. The process of claim 8 or 9 wherein at least two stretching stages are performed on the xerogel.

11. The process of any previous claim wherein the stretching is performed in at least two stages with the latest stage performed at a temperature of between 130°C and 230°C.

12. The process of any previous claim wherein said polyacrylonitrile has a weight average molecular weight of at least 750,000.

13. The process of any previous claim wherein said cooling step (c) includes immersing the solution in a quench bath containing a mixture of first solvent and water at a temperature of 0°C to 50°C.

14. A polyacrylonitrile fiber of weight average molecular weight at least 500,000 and having a tenacity of at least 5 g/denier (44.1 cN/tex) and a secant modulus of at least 100 g/denier (882 cN/tex).

15. The polyacrylonitrile fiber of claim 14 being of weight average molecular weight of at least 750,000.

16. The polyacrylonitrile fiber of claim 14 or 15 having a tenacity of at least 7 g/denier (61.74 cN/tex) and a secant modulus of at least 125 g/denier (1102.5 cN/tex).

17. The polyacrylonitrile fiber of claim 14 or 16 being of weight average molecular weight of between 1,000,000 and 4,000,000.

## Patentansprüche

1. Gelspinnverfahren zur Herstellung von Polyacrylnitrilfaser, umfassend folgende Stufen:
(a) Herstellung einer Lösung aus im wesentlichen linearen Polyacrylnitril mit einem gewichtsmittleren Molekulargewicht von mindestens 500 000 in einem ersten Lösungsmittel bei einer ersten Konzentration von 2 bis 15 Gewichtsprozent Polyacrylnitril und bei einer ersten Temperatur oberhalb der Geliertemperatur des besagten Lösungsmittels mit einem Dampfdruck von höchstens 80 kPa bei diesen ersten Temperatur,
(b) Extrusion dieser Lösung durch eine Öffnung in eine Gasatmosphäre, wobei sich die extrudierte Lösung bei einer Temperatur über der Geliertemperatur befindet und die Polyacrylnitrilkonzentration sowohl vor als auch nach dieser Öffnung im wesentlichen der ersten Konzentration entspricht,
(c) Abkühlung der Lösung in einer Kühlzone anschliessend an die und hinter der Gasatmosphäre auf eine zweite Temperatur unterhalb der Geliertemperatur zur Bildung eines gummiartigen, erstes Lösungsmittel enthaltenden Gels weitegehend unendlicher Länge,
(d) Extraktion des erstes Lösungsmittel enthaltenden Gels mit einem zweiten Lösungsmittel, das leichtflüchtiger als jenes erste Lösungsmittel ist, für einen genügenden Zeitraum, um eine zweites Lösungsmittel enthaltende faserartige Struktur zu bilden, welche im wesentlichen frei von erstem Lösungsmittel ist und eine weitegehend unendliche Länge aufweist,
(e) Trocknung der zweites Lösungsmittel enthaltenden Faserstruktur zu einem Xerogel weitgehend unendlicher Länge, des frei von erstem und zweitem Lösungsmittel ist, und
(f) Reckung mindestens eines von:
(i) dem erstes Lösungsmittel enthaltenden Gel,
(ii) der zweites Lösungsmittel enthaltenden Faserstruktur und
(iii) dem Xerogel bei einem genügenden Gesamtreckverhältnis, um eine Reissfestigkeit von mindestens 5 g/denier (44,1 cN/tex) und einen Sekantenmodul von mindestens 100 g/denier (882 cN/tex) zu erreichen.

2. Verfahren nach Anspruch 1, worin die besagte Öffnung einen im wesentlichen kreisförmigen Querschnitt aufweist, das besagte erstes Lösungsmittel enthaltende Geleine Gel faser ist und das besagte Xerogel eine Xerogelfaser ist.

3. Verfahren nach Anspruch 1 oder 2, worin die besagte erste Temperatur zwischen 130°C und 250°C sowie besagte zweite Temperatur zwischen 0°C und 50°C liegt und die Abkühlungsgeschwindigkeit zwischen jener ersten und zweiten Temperatur mindestens 50°C/Minute beträgt.

4. Verfahren nach einem der vorhergehenden Ansprüche, worin besagtes zweites Lösungsmittel einen atmosphärischen Siedepunkt von 100°C oder niedriger besitzt.

5. Verfahren nach einem der vorhergehenden Ansprüche, worin besagtes erstes Lösungsmittel aus der Dimethylsulfoxid, Dimethylformamid, Dimethylacetamid, gamma-Butyrolacton und Äthylencarbonat umfassenden Gruppe ausgewählt ist.

6. Verfahren nach einem der Ansprüche 1 bis 3, worin als besagtes erstes Lösungsmittel Dimethylsulfoxid vorliegt, die besagte erste Temperatur bei 130°C bis 200°C liegt und besagte erste Konzentration 5 bis 8 Gew-% beträgt.

7. Verfahren nach einem der vorhergehenden Ansprüche, worin besagte Reckstufe (f) in mindestens zwei Schritten durchgeführt wird.

8. Verfahren nach Anspruch 7, worin beim ersten Schritt das erstes Lösungsmittel enthaltende Gel gereckt wird.

9. Verfahren nach Anspruch 8, worin beim zweiten Schritt das Xerogel gereckt wird.

10. Verfahren nach Anspruch 8 oder 9, worin mindestens zwei Reckschritte am Xerogel durchgeführt werden.

11. Verfahren nach einem der vorhergehenden Ansprüche, worin die Reckung im mindestens zwei Schritten erfolgt, wobei der letzte Schritt bei einer Temperatur zwischen 130°C und 230°C durchgeführt wird.

12. Verfahren nach einem der vorhergehenden Ansprüche, worin besagtes Polyacrylnitril ein gewichtsmittleres Molekulargewicht von mindestens 750 000 besitzt.

13. Verfahren nach einem der vorhergehenden Ansprüche, worin es sich bei besagter Kühlstufe (c) um das Eintauchen der Lösung in ein Abschreckbad handelt, das ein Gemisch aus erstem Lösungsmittel und Wasser bei einer Temperatur von 0°C bis 50°C enthält.

14. Polyacrylnitrilfaser mit einem gewichtsmittleren Molekulargewicht von mindestens 500 000, einer Reissfestigkeit von mindestens 5 g/denier (44,1 cN/tex) und einem Sekantenmodul von mindestens 100 g/denier (882 cN/tex).

15. Polyacrylnitrilfaser nach Anspruch 14 mit einem gewichtsmittleren Molekulargewicht von mindestens 750 000.

16. Polyacrylnitrilfaser nach Anspruch 14 oder 15 mit einer Reissfestigkeit von mindestens 7 g/denier (61,74 cN/tex) und einem Sekantenmodul von mindestens 125 g/denier (1102,5 cN/tex).

17. Polyacrylnitrilfaser nach Anspruch 14 oder 16 mit einem gewichtsmittleren Molekulargewicht zwischen 1 000 000 und 4 000 000.

## Revendications

1. Un procédé de filage de gel pour préparer une fibre de polyacrylonitrile comprenant les étapes suivantes:
(a) former une solution d'une polyacrylonitrile sensiblement linéaire ayant un poids moléculaire pondéral moyen d'au moins 500.000 dans un premier solvent à une première concentration de 2 à 15 pour-cent en poids de polyacrylonitrile, et à une première température supérieure à la température de gélification, ledit solvant ayant une tension de vapeur ne dépassant pas 80 kPa à ladite première température,
(b) extruder ladite solution à travers un orifice dans une atmosphère gazeuse, la solution extrudée étant à une température supérieure à la température de gélification et la concentration en polyacrylonitrile étant sensiblement à la première concentration aussi bien en amont qu'en aval dudit orifice,
(c) refroidir la solution dans une zone de refroidissement adjacente à et en aval de l'atmosphère gazeuse jusqu'à une seconde température inférieure à la température de gélification pour former un gel caoutchouteux contenant le premier solvent, et de longueur sensiblement non-définie,
(d) extraire le gel contenant le premier solvant à l'aide d'un second solvant qui est plus volatil que ledit premier solvant pendant un temps de contact suffisant pour former une structure fibreuse contenant le second solvant, laquelle structure fibreuse est sensiblement dépourvue de premier solvant et est de longueur sensiblement non-définie.
(e) sécher la structure fibreuse contenant le second solvant pour former un xérogel de longueur sensiblement non-définie, dépourvu de premier et de second solvants, et
(f) étirer au moins l'un des suivants:
(i) le gel contenant le premier solvant,
(ii) la structure fibreuse contenant le second solvant, et
(iii) le xérogel, à un rapport d'étirage total suffisant pour obtenir une ténacité d'au moins 5 g/denier (44,1 cN/tex) et un module sécant d'au moins 100 g/denier (882 cN/tex).

2. Le procédé selon la revendication 1 dans lequel ledit orifice a une section transversale sensiblement circulaire; ledit gel contenant le premier solvant est une fibre gel et ledit xérogel est une fibre xérogel.

3. Le procédé selon la revendication 1 ou 2 dans lequel ladite première température est comprise entre 130°C et 250°C; ladite seconde température est comprise entre 0°C et 50°C; et la vitesse de refroidissement entre ladite première température et ladite seconde température est d'au moins 50°C/mn.

4. Le procédé selon l'une quelconque des revendications précédentes dans lequel ledit second solvant a un point d'ébullition à la pression atmosphérique de 100°C ou inférieur.

5. Le procédé selon l'une quelconque des revendications précédentes dans lequel ledit premier solvant est choisi parmi le groupe constitué du diméthylsulfoxyde, du diméthylformamide, du diméthylacétamide de la gammabutyrolactone et du carbonate d'éthylène.

6. Le procédé selon l'une quelconque des revendications 1-3 dans lequel ledit premier solvant est le diméthylsulfoxyde, ladite première température est de 130°C à 200°C et ladite première concentration est de 5 à 8 pourcent en poids.

7. Le procédé selon l'une quelconque des revendications précédentes dans lequel ladite étape d'étirage (f) est effectuée en au moins deux stades.

8. Le procédé selon la revendication 7 dans lequel un premier stade d'étirage est celui du gel contenant le premier solvant.

9. Le procédé selon la revendication 8 dans lequel un seconde stade d'étirage est celui du xérogel.

10. Le procédé selon la revendication 8 ou 9 dans lequel on effectue au moins deux stades d'étirage sur le xérogel.

11. Le procédé selon l'une quelconque des revendications précédentes dans lequel on effectue l'étirage en au moins deux stades, le dernier stade étant effectué à une température comprise entre 130°C et 230°C.

12. Le procédé selon l'une quelconque des revendications précédentes dans lequel ledit polyacrylonitrile a un poids moléculaire pondéral moyen d'au moins 750.000.

13. Le procédé selon l'une quelconque des revendications précédentes, dans lequel ladite étape de refroidissement (c) inclut l'immersion de la solution dans un bain de trempe contenant un mélange de premier solvent d'eau à une température de 0°C à 50°C.

14. Une fibre de polyacrylonitrile de poids moléculaire pondéral moyen d'au moins 500.000 et ayant une ténacité d'au moins 5 g/denier (44,1 cN/tex) et un module sécant d'au moins 100 g/denier (882 cN/tex).

15. La fibre de polyacrylonitrile selon la revendication 14 ayant un poids moléculaire pondéral moyen d'au moins 750.000.

16. La fibre de polyacrylonitrile selon la revendication 14 ou 15 ayant une ténacité d'au moins 7 g/denier (61,74 cN/tex) et un module sécant d'au moins 125 g/denier (1102,5 cN/tex).

17. La fibre de polyacrylonitrile selon la revendication 14 ou 16 ayant un poids moléculaire pondéral moyen compris entre 1.000.000 et 4.000.000.
